

J. H. BAMBERG,  
PISTON CASTING,  
APPLICATION FILED MAR. 6, 1917.

1,296,592.

Patented Mar. 4, 1919.

2 SHEETS—SHEET 1.



WITNESS:

Russel N. Dow

INVENTOR.

Joseph H. Bamberg  
BY  
Ray A. Gehr  
ATTORNEY.

J. H. BAMBERG.  
PISTON CASTING.  
APPLICATION FILED MAR. 6, 1917.

1,296,592.

Patented Mar. 4, 1919.

2 SHEETS—SHEET 2.



WITNESS:

Russel N. Dow

INVENTOR.

Joseph H. Bamberg  
BY

Ray S. Lehr

ATTORNEY.

# UNITED STATES PATENT OFFICE.

JOSEPH H. BAMBERG, OF TOLEDO, OHIO, ASSIGNOR TO THE ALUMINUM CASTINGS COMPANY, OF CLEVELAND, OHIO, A CORPORATION OF OHIO.

## PISTON-CASTING.

1,296,592.

Specification of Letters Patent.

Patented Mar. 4, 1919.

Original application filed March 7, 1916, Serial No. 82,529. Divided and this application filed March 6, 1917. Serial No. 152,896.

*To all whom it may concern:*

Be it known that I, JOSEPH H. BAMBERG, a citizen of the United States, residing at Toledo, in the county of Lucas and State of Ohio, have invented certain new and useful Improvements in Piston-Castings, of which the following is a specification, reference being had therein to the accompanying drawing.

10 This invention relates to an internal combustion motor piston casting having internally projecting bosses, webs, ribs and extensions, or either of them.

One object of my invention is to provide a 15 skirted piston cast of metal or metallic alloy of relatively low specific gravity and which is relatively non-porous, free from entrapped air and other gases and oxids and other foreign materials.

20 Another object of my invention is to provide a skirted piston cast of metal or metallic alloy of relatively low specific gravity and readily machinable to provide durable and efficient bearing surfaces.

25 Another object of my invention is to provide a casting for a skirted piston for an internal combustion motor made from metal or metallic alloy of relatively low specific gravity and having different structural characteristics at various sections as desired.

30 Another object of my invention is to provide a skirted piston casting of metallic alloy having a relatively low specific gravity and a relatively high coefficient of heat 35 conductivity, which when machined and used in the cylinder of an internal combustion motor will not collect carbon to the same extent as does an iron piston and will take and retain a relatively high polish because 40 of its fine-grained structure.

Another object of this invention is to provide a skirted piston casting made of a minimum volume of metallic alloy of relatively low specific gravity and high heat 45 conductivity, which will not disintegrate nor undergo changes in its internal structure under ordinary usage in an internal combustion motor, and which will require a minimum amount of machining.

50 Another object of my invention is to provide a skirted piston casting made of a metallic alloy of relatively low specific gravity and high heat conductivity and in which casting there is a relatively small amount of

eutectic which substantially surrounds the 55 excess substance in the casting.

Another object of my invention is to provide a skirted piston casting made of an alloy of relatively low specific gravity and high heat conductivity and in which casting 60 there is a relatively small amount of eutectic disposed relative to the excess substance in such manner as to provide efficient and durable machined bearing surfaces.

Another object of this invention is to provide a piston casting of an alloy containing aluminum, tin and copper, having a structure relatively fine-grained, non-porous and free from entrapped air and other gases and from oxids and other foreign materials.

65 Other objects of my invention will be obvious to one skilled in the art from the description of it hereinafter made.

70 The present application is a division of my pending application, Serial No. 82,529, filed March 7, 1916, in which I have fully set forth and explained an apparatus and method suitable for the production of the piston casting to which the present application relates.

75 In order that the present invention may be clearly understood, I have shown in the accompanying drawings one form of piston casting embodying my improvements and also a mold in which the casting is 80 formed.

Figure 1 is a perspective view of a skirted or cup-shaped piston casting, after the sprue has been removed.

85 Fig. 2 is a central longitudinal sectional view through the piston casting.

Fig. 3 is a central longitudinal sectional view of the piston casting taken at right angles to the section shown in Fig. 2.

90 Fig. 4 is a bottom plan view of the piston casting.

Fig. 5 is a side elevation of a mold adapted for the production of my improved piston casting, part of the view being in section and the core pins being shown removed.

100 Fig. 6 is a top plan view of the mold with the mold members separated and the casting attached to one of them.

The piston casting, as to outward formation, has the usual piston head 1 and side wall 2 characteristic of the skirted pistons commonly employed in internal combustion engines. The side wall is formed with dia-

metrically opposite inwardly projecting bosses 3, 3 which are cored out to receive a wrist-pin. The upper part of the casting, as shown, is provided with strengthening 5 and heat-dissipating ribs 4 and 5.

My improvements are not limited to the particular conformation of the casting shown but may be varied widely, as will be understood from the following explanation 10 of the matters which characterize my improvements.

The physical properties and internal structural characteristics which chiefly characterize my invention are the result of the constituent materials employed in the casting and the manner in which the casting is formed. I will, accordingly, briefly describe a mold designed for the production of the casting and the manner in which such mold 20 is used. For a full description and explanation of the mold and the process of producing the casting by means of it, reference is had to my pending application, Serial No. 82,529, above referred to.

25 Referring to Figs. 5 and 6, the mold comprises a base member *a* and complementary members *b* and *c*, movable on the base member *a* toward and from each other. *d* indicates as an entirety the main core part of the 30 mold. This core is formed in a plurality of sections which are suitably recessed to form the bosses 3, 3 and ribs 4 and 5 on the interior of the piston. *e*, *e* are diametrically opposite core pins arranged to project into 35 the mold cavity to form openings in or through the bosses 3, 3 of the piston casting. These core pins are in the form of rods which are slidably mounted in alining openings of the mold members *b* and *c*.

40 The mold members *b* and *c* are formed with complementary cavities or recesses *b'* and *c'* which together form the mold gate. The gate thus formed, as will be observed from Fig. 6, is disposed midway between 45 the internal bosses 3, 3 of the piston casting. As is fully explained in my co-pending application referred to, I prefer to employ a gate constructed so that a liquid seal is formed which precludes the passage of air 50 and gases into the mold cavity and also materially reduces splashing of metal within the gate during the pouring. Also the gate is preferably formed to communicate with the mold cavity at the bottom and at 55 the top of the cavity and at intermediate points between the top and bottom.

The walls of the mold cavity are suitably coated or treated, in any well-known manner, to reduce as much as possible agitation 60 of the molten metal as it flows into contact therewith, and to insure proper setting of the metal within the mold cavity and a free separation of the casting from the mold. The inner walls of the cavity are also 65 formed so as to provide for venting of the

cavity to assure the ready escape of air or gases as the molten metal flows in.

Suitable means are provided for heating the walls of the mold members *b*, *c*, and as the main core *d* and the core pins *e*, *e* are 70 separable from the members *b*, *c*, said parts *d* and *e* may readily be maintained at desired temperatures. As I have fully explained in my application, Serial No. 82,529, the core pins are preferably kept at a temperature substantially lower than the other parts of the mold cavity walls, and the temperature of the gate walls is kept higher than the other parts of members *b* and *c*; and consequently when the molten metal, at 75 a temperature hundreds of degrees above the temperatures of the mold walls, is poured into the mold cavity it is subjected to a very strong chilling action at points adjacent the core pins *e*, *e* and to a less marked but very 80 substantial chilling action adjacent other parts of the cavity walls, while the higher temperature of the gate walls insures the maintenance of molten metal in the gate until after freezing takes place in the mold 85 cavity so that crystallization shrinkage of the casting proper is obviated by the molten gate metal.

90 My invention, in its broader aspects, is not limited to the use of any one metal or 95 metallic alloy for the casting; in fact, my co-pending application, above referred to, mentions several metallic alloys which can be used advantageously in the carrying out of the invention. Certain metallic alloys, however, have peculiar advantages and adaptability for the production of castings to meet particular requirements, and the present application relates more especially to a piston casting formed of an aluminum alloy containing 100 tin and copper. While the proportions of these constituents may be varied somewhat, I prefer an alloy having approximately the following composition: aluminum 94.0 to 94.5%, copper 5.0% and tin 1.0 105 to 0.5%.

110 In making a piston casting of metallic allow such as last referred to, the molten metal, at a suitable temperature between 1350° F. and 1400° F., is poured by gravity 115 through the gate and into the cavity of the mold. The first of the molten metal entering the mold cavity fills the bottom thereof (this part of the cavity corresponding to the head of the piston) and thereafter the molten 120 metal, as it enters the mold cavity, flows from the gate opening in opposite directions around the upright cylindrical parts of the cavity, the level of the metal in the cavity gradually rising until the cavity is 125 filled. And, correspondingly, the metal of the casting freezes progressively from the bottom upward and from the side of the mold cavity opposite the gate toward the gate. When a brief interval after the pour- 130

ing has elapsed, usually as soon as the crystallization shrinkage occurs, the core pins *e, e* are withdrawn; and then after a suitable further interval the core *d* is removed, 5 the mold members *b, c* are separated and the casting removed.

The chilling effect of the different parts of the cavity walls upon the metal of the casting, when the casting is of a suitable composition and suitably poured in the manner referred to, gives to the casting physical properties and internal structural characteristics which are remarkable and, as I believe, greatly superior to any which have heretofore been obtained.

These superior properties and characteristics of my improved piston castings are: low specific gravity, high coefficient of heat conductivity, relatively great strength, and 10 a non-porous fine grained structure free from impurities and from cavities due to crystallization shrinkage and with the eutectic substantially surrounding the excess material in such manner as to provide a 15 durable and efficient bearing surface when the casting is machined. Furthermore the casting, with an internal structure such as described, has very excellent machining qualities, while, both because of its structural character and the accuracy with which 20 it is formed, little machining is required in producing the finished piston. Again the structure of the metal of the inner walls of the bosses *3, 3*, resulting from the relatively 25 quick setting of said metal, is particularly 30 advantageous for co-operation with the wristpin.

By reason of its fine grained, dense structure the casting, when machined, takes a 35 high polish and has less tendency to collect 40 carbon than does an iron piston. I have mentioned the bearing and wearing qualities of the casting and, in that connection may add that I have been unable to note any 45 disintegration in the structure of these castings 50 after thousands of miles of severe service in relatively high speed motors of the internal combustion type. Furthermore, the internal 55 physical structure of the casting characteristic of the above mentioned relation of the eutectic and excess substance is not changed by the working temperatures of the internal combustion motor to which said castings are subjected.

55 With respect to the relation of the eutectic and excess substance in my improved castings, I may observe that while the eutectic substantially surrounds the excess substance as stated above, I believe it is desirable that

it should not entirely surround and completely isolate said excess substance; for, by avoiding such complete isolation of the excess substance, I believe greater tensile strength is secured.

To those skilled in the art many modifications of and widely differing embodiments and applications of my invention will suggest themselves, without departing from the spirit and scope thereof. My disclosures and the descriptions herein are purely illustrative and are not intended to be in any sense limiting.

What I claim is:

1. As a new article of manufacture, an internal combustion motor piston casting 75 made of an alloy consisting predominantly of aluminum and containing tin and copper, the casting having chilled walls and being fine grained and substantially free from porosity due to crystallization shrinkage.

2. As a new article of manufacture, an internal combustion motor piston casting made of an alloy consisting predominantly of aluminum and containing other elements such as tin and copper in proportions to produce a relatively small quantity of eutectic in the casting after freezing, the casting having the said eutectic substantially surrounding the excess substance therein and having 85 chilled walls.

3. As a new article of manufacture, an internal combustion motor piston casting made of an alloy consisting predominantly of aluminum and containing other elements such as tin and copper in proportions to 90 produce a relatively small quantity of eutectic in the casting after freezing, the casting having the said eutectic substantially surrounding the excess substance therein and being fine grained and substantially free 95 from porosity due to crystallization shrinkage.

4. As a new article of manufacture, an internal combustion motor piston casting made of an alloy consisting predominantly of aluminum and containing other elements such as tin and copper in proportions to produce a relatively small quantity of eutectic in the casting after freezing, the casting having the said eutectic substantially surrounding the excess substance therein and being fine grained and substantially free 100 from porosity due to crystallization shrinkage.

In testimony whereof, I hereunto affix my 115 signature.

JOSEPH H. BAMBERG.